

# United States Patent [19]

Takegawa et al.

[11] 3,816,132

[45] June 11, 1974

[54] **HEAT-DEVELOPABLE LIGHT-SENSITIVE MATERIALS**

[75] Inventors: **Yukio Takegawa; Takao Matui; Tetuya Higuchi**, all of Tokyo, Japan

[73] Assignee: **Oriental Photo Industrial Co., Ltd.**, Tokyo, Japan

[22] Filed: **Mar. 22, 1973**

[21] Appl. No.: **343,867**

[30] **Foreign Application Priority Data**

Mar. 27, 1972 Japan ..... 47-30568

[52] U.S. Cl. ..... **96/48 HD, 96/50 PT, 96/67, 96/94 R, 96/114, 96/114.1**

[51] Int. Cl. ..... **G03c 1/60, G03c 1/72**

[58] **Field of Search** ..... **96/114.1, 48 HD, 94 R, 96/67, 50 PT**

[56]

## References Cited

### UNITED STATES PATENTS

3,764,329 10/1973 Lee ..... 96/67

*Primary Examiner*—Ronald H. Smith

*Assistant Examiner*—Alfonso T. Suro Pico

*Attorney, Agent, or Firm*—Woodhams, Blanchard and Flynn

[57]

## ABSTRACT

A heat-developable light-sensitive material containing no silver halide is provided. An image-forming ability is imparted to the material by activating the heat-developable light-sensitive reproducing material containing at least a silver salt of long chain fatty acid, an organic reducing agent and an organic carboxylic acid by means of a heat pre-treatment.

16 Claims, No Drawings

## HEAT-DEVELOPABLE LIGHT-SENSITIVE MATERIALS

### BACKGROUND OF THE INVENTION

#### 1. Field of the Invention

The present invention relates to a heat-developable light-sensitive material. More particularly, the invention relates to a heat-developable light-sensitive material containing no silver halide, the sensitivity and image densities of which have been highly improved by subjecting the material to a suitable heat pre-treatment.

#### 2. Description of the Prior Art

Known silver halide photography is superior to other various photographic techniques with respect to sensitivity, gradient, etc. However, its treatment steps such as development and fixing steps are troublesome, since they are carried out in the wet system, and it is inconvenient to mechanize the whole steps in many aspects.

Many attempts have been made for improving the silver halide photography by converting its treatment steps from the wet system to the dry system.

Among them, heat-developable light-sensitive materials which are to be developed by heat treatment have been proposed in patent literatures. In Japanese Patent Publication No. 4924/1968 (Belgian Patent No. 663,112; French Patent No. 1,441,691; OLS 1,572,203; British Patent No. 1,110,046), there has been disclosed a heat-developable light-sensitive material consisting of an organic silver salt, a reducing agent and a silver halide catalytically contacted with said organic silver ion. In said Japanese Patent Publication No. 4924/1968, there is described an example as control in which no halogen donor is used. In this example, a system comprising an organic silver salt, a reducing agent, a binder and an acidic stabilizer is exposed to the pattern of an image and then heat-developed to obtain only a faint gray image on slight turbid yellow back. It is also described therein that no practically advantageous image density could be obtained even by changing exposure conditions and heat-developing conditions.

### SUMMARY OF THE INVENTION

We have found that a heat-developable light-sensitive material capable of producing an effective image density can be obtained by forming a single layer or multilayers containing a silver salt of long chain fatty acid, an organic reducing agent and an organic carboxylic acid, preferably on a support, and then subjecting the same to a heat pretreatment under proper heating conditions to impart an excellent light sensitivity to said material, which can never be obtained without such heat pre-treatment.

Although the detailed mechanism of imparting light sensitivity to the system not containing light-sensitive silver halide to make the formation of an image of effective image density possible is not yet known, a possible explanation is as follows:

By the heat pre-treatment according to the present invention, the silver salt of long chain fatty acid which is hardly dissociated at ambient temperature may be partially thermally dissociated to release silver ion. Thus, the resulted silver ion may form a neutral silver aggregate which is capable of acting as sensitivity speck in the successive exposure step. Another possible ex-

planation is as follows: By the heat pre-treatment according to the present invention, the organic acid is molten and thereby acts as a solvent, which may facilitate to melt and dissociate the silver salt of long chain fatty acid. The dissociated silver ion forms a sensitivity speck according to the above assumed mechanism.

Although the above mechanisms have not been proved yet, it cannot but be considered to be a surprising, quite important finding that a silver salt of long chain fatty acid which has been considered to be non-sensitive or practically non-sensitive can be converted to a useful light-sensitive material by the heat pre-treatment according to the present invention.

Description will be made on the process for the preparation of the heat-developable light-sensitive materials of the present invention and the process for the formation of an image in said materials.

According to a preferred embodiment of the present invention, the first coating layer comprising a silver salt of long chain fatty acid and an organic carboxylic acid dispersed in a binder material is provided on a support made of such materials as paper, etc. Then, the surface of the layer is treated with a treating solution containing a reducing agent and thereafter dried. However, at this step, the product hardly has any image-forming property. Then, it is subjected to a heat pre-treatment for a proper time at a temperature, at which a part of the silver salt in the system may be dissociated. Thus, an excellent light sensitivity is obtained. The light-sensitive material thus obtained is exposed to the pattern of an image and then heat-developed at a temperature higher than that of the heat pre-treatment. By this treatment, a silver image is formed selectively in the exposed portion by the action of the reducing agent contained therein. As the energy source for the exposure, ultraviolet rays or another radiation energy may be used in addition to visible rays.

As clearly shown by the above described process for the preparation and process for the formation of an image, the light-sensitive material of the present invention hardly has light-sensitivity before the heat pre-treatment and, therefore, it may be exposed to ordinary indoor lights for a short time. Further, by adding mercury salts which will be described below as anti-foggant, the light-sensitivity prior to the heat pre-treatment can be inhibited completely. Namely, no particular light-intercepting means is required at the time of packing, storage or transportation, if the material is passed through a heating roll or subjected to another heat pre-treatment immediately before the material is to be introduced in a successive exposure device.

The sensitivity imparted to the material by the heat pre-treatment is not substantially extinguished as time elapses. This property is utterly different from the phenomenon that the sensitivity caused by the electric charge extinguishes as time elapses in electrophotography. However, the sensitivity is inclined to be gradually extinguished if the material is placed in an atmosphere containing vapor of a solvent which is capable of swelling and dissolving the coated material. Therefore, for preventing the reduction of the sensitivity, it is preferred to avoid the use of atmosphere of a solvent such as trichloroethylene, toluene, acetone and alcohol. On the contrary, for promoting the reduction of sensitivity intentionally, the material may be exposed to the atmosphere of such solvents.

As silver salts used in the present invention, there may be mentioned silver salts of organic acids or silver salts of organic compounds containing imide group or mercapto group. Particularly, those which are hardly deteriorated or darkened at room temperature under indoor light are silver salts of long chain fatty acids such as silver behenate, silver stearate, silver palmitate, silver myristate, silver laurate, silver oleate and silver hydroxystearate. Silver salts of fatty acids having 18 – 24 carbon atoms are preferable.

As reducing agents used in the present invention, there may be mentioned aromatic compounds substituted with hydroxyl group. Particularly effective compounds are hydroquinone, methylhydroquinone, chlorohydroquinone, bromohydroquinone, catechol, pyrogallol, methylhydroxynaphthalene, aminophenol, 2,2'-methylene-bis(6-tert.-butyl-4-methylphenol), 4,4'-butylidene-bis(6-tert.-butyl-3-methylphenol), 4,4'-thiobis(6-tert.-butyl-2-methylphenol), etc. Furthermore, amino compounds such as N,N'-diethyl-p-phenylenediamine and N-phenyl-N'-isopropyl-p-phenylenediamine are also effective. In addition, bis-naphthol reducing compounds described in U.S. Pat. No. 3,672,904 (French Patent No. 2,090,923; Belgian Patent No. 766,589) are also effective. Those compounds may be used singly or in combination.

Suitable organic carboxylic acids used in the present invention are aliphatic monocarboxylic acids, aliphatic unsaturated monocarboxylic acids, dicarboxylic acids and aromatic carboxylic acids. There may be mentioned, for example, capric acid, lauric acid, palmitic acid, stearic acid, arachidic acid, behenic acid, lignoceric acid, cerotic acid, linolic acid, oleic acid, succinic acid, adipic acid, sebacic acid, benzoic acid, cinnamic acid, salicylic acid, p-hydroxybenzoic acid, 2,6-dihydroxybenzoic acid, phthalic acid, isophthalic acid, trimellitic acid, pyromellitic acid, diphenic acid, 5,5'-methylene-bis-salicylic acid, tetrachlorobenzoic acid and tetrabromobenzoic acid. Particularly, long chain fatty acids having 18 to 24 carbon atoms are preferable.

Optimum temperature range and heating time of the heat pre-treatment which is one of characteristic features of the present invention depend on the kinds of silver salt of long chain fatty acid, organic reducing agent and organic carboxylic acid used. In this heat pre-treatment, it is desirable that as much as the amount of heat should be supplied to the material within the limit of substantially causing no fog on the material, that is, the change in optical density of the surface of the material during the heat-pre-treatment being less than 0.1. Generally, the heat treatment can be carried out at a temperature of 50° – 200°C. Preferably, the heat pretreatment should be effected at 70° – 120°C for a short period of time. For example, when a system comprising a combination of silver behenate, 2,2'-methylene-bis(6-tert.-butyl-4-methylphenol) and behenic acid is employed as in Example 3 which will be given below, it is preferred to carry out the heat treatment at 80°C for 5 – 30 seconds or at 100°C for 1 – 5 seconds. Heating for a longer period of time is undesirable, since it causes fog.

A preferred heat pre-treatment comprises heating the surface of a support which was coated with a dispersion of a silver salt of long chain fatty acid and an organic carboxylic acid in a suitable binder and treated with a solution of a reducing agent in a suitable solvent,

with a heating roll, heating plate or hot air at the time of drying or at a suitable time after the drying but before the exposure.

The light-sensitive material of the present invention 5 may be added with a toning agent, an antifoggant etc., depending upon the kinds of silver salt or reducing agent used. For example, phthalazinone and derivates thereof described as toning agents for heat sensitive reproducing paper containing a silver salt of long chain fatty acid in U.S. Pat. No. 3,080,254 are effective toning agents. Further, cyclic imides disclosed in U.S. Pat. No. 3,672,904 are also effective toning agents. Mercury salts described in U.S. Pat. No. 3,589,903 are effective as antifoggant, storage stabilizer and toning agent. White pigments such as zinc oxide, titanium dioxide, etc. have effects of improving whiteness of the back (non-image part) and also of improving image density and apparent sensitivity.

The light-sensitive material of the present invention 20 can be sensitized by incorporating therein a spectral sensitizing dye selected from the class consisting of cyanines, merocyanines oxonols and acridines. Though it is said that Acridine Yellow have no sensitizing effect to silver halides, it can also be used in the present invention.

A binder may be preferably incorporated in the light-sensitive material of the present invention.

As suitable binders, there may be mentioned polyvinyl butyral, cellulose acetate butyrate, polymethyl methacrylate, polyvinyl pyrrolidone, ethylcellulose, cellulose acetate, cellulose acetate butyrate, polyvinyl acetate, polyvinyl alcohol and gelatin.

In preparing the light-sensitive material of the present invention, there is preferably used a support or a base. Any material which is stable against heating may be used. Suitable supports or bases are films of synthetic resins such as polyethylene terephthalate, polycarbonate and cellulose acetate; foils of metals such as 35 aluminum; and various kinds of papers.

Optimum ratio of the components of the present invention depends upon the kinds of silver salt of long chain fatty acid, reducing agent and organic carboxylic acid used. In general, it is proper to use 10 – 0.01 part 45 by weight of an organic reducing agent and 10 – 0.01 part by weight of an organic carboxylic acid per 1 part by weight of a silver salt of long chain fatty acid. Preferably, 1 – 1/10 mole of an organic reducing agent and 10 – 1/10 mole of an organic carboxylic acid are used 50 per mole of a silver salt of long chain fatty acid.

It will be easily understood by those skilled in the art that in place of the heat pre-treatment of the above coating composition, a selective heat image may be applied followed by the whole surface exposure and heat development for the purpose of heat-sensitive reproduction.

The present invention will now be illustrated by way of examples.

#### Example 1

The first coating dispersion of the following composition was applied to a photographic base paper by using a roll coater and then dried. Amount of the coating was 12 g per m<sup>2</sup> of the base after drying.

-Continued

|                   |        |
|-------------------|--------|
| Behenic acid      | 13 g   |
| Polyvinyl butyral | 40 g   |
| Toluene           | 350 ml |
| Ethanol           | 350 ml |

5

Then, the second coating solution containing a reducing agent of the following composition was applied by using a roll coater and dried at a temperature below 50°C. Amount of the coating was 1.0 g per m<sup>2</sup> of the base after drying.

10

|                   |         |
|-------------------|---------|
| Hydroquinone      | 30 g    |
| Polyvinyl butyral | 10 g    |
| Methanol          | 1000 ml |

15

The thus resulting coating composition was subjected to heat pre-treatment with a heating roller at 90°C for 5 seconds and then exposed to the light of blue luminescent lamp (Toshiba FL-20B) through a negative image. Then, it was heated for development at 105°C for 5 seconds to obtain a dark brown positive image.

20

#### Example 2

Coating compositions were prepared in the same manner as in Example 1, except using an equimolar amount of sebacic acid in place of behenic acid and 23 g of N-phenyl-N'-isopropyl-p-phenylene-diamine in place of hydroquinone reducing agent in the second coating liquid. These coating compositions were applied to the same base paper in the same manner as in Example 1. After heat pre-treatment, exposure and heat development in the same manner as in Example 1, a dark brown positive image was obtained. Suitable heating conditions of the heat pre-treatment and heat development in this case were 80°C for 5 seconds and 100°C for 5 seconds, respectively.

25

#### EXAMPLE 3

A heat developable light-sensitive material was prepared in the same manner as in Example 1, except that the second coating solution of the following composition was used. The amount of the coating was 2.5 g per m<sup>2</sup> of the base after drying.

30

|                                                  |         |
|--------------------------------------------------|---------|
| 2,2'-methylene-bis(6-tert.-butyl-4-methylphenol) | 100 g   |
| Phthalazinone                                    | 5 g     |
| Polyvinyl butyral                                | 10 g    |
| Methanol                                         | 1000 ml |

35

The obtained material was subjected to heat pre-treatment by using a heat roller for 5 seconds and then to step exposure by using a blue luminescent lamp as light source through Kodak Step Tablet No. 2. Thereafter, heating was effected at 105°C for 5 seconds. The samples subjected to the heat pretreatment yielded a mild black image depending upon the amount of exposure. The relations between heat pre-treatment temperatures and the resulting image characteristics are shown in the following Table.

40

\*Sensitivity is represented by number of steps of tablet which gives a density of 0.1 above the fog.

\*\*Dm and Df represent the image maximum density and fog density, respectively.

45

#### EXAMPLE 4

The first coating dispersion and the second coating solution of the following compositions were applied to a photographic base paper in this order and then dried.

50

##### First coating dispersion:

|                   |        |
|-------------------|--------|
| Silver stearate   | 15 g   |
| Stearic acid      | 11 g   |
| Polyvinyl butyral | 20 g   |
| Toluene           | 300 ml |
| Ethanol           | 300 ml |

##### Second coating solution:

|                                                  |         |
|--------------------------------------------------|---------|
| 2,2'-methylene-bis(6-tert.-butyl-4-methylphenol) | 100 g   |
| Phthalazinone                                    | 5 g     |
| Polyvinyl butyral                                | 10 g    |
| Methanol                                         | 1000 ml |

55

##### First coating dispersion:

|                   |        |
|-------------------|--------|
| Silver behenate   | 17 g   |
| Behenic acid      | 13 g   |
| Mercuric acetate  | 0.12 g |
| Polyvinyl butyral | 40 g   |
| Toluene           | 350 ml |
| Ethanol           | 350 ml |

##### Second coating solution:

|                                                  |         |
|--------------------------------------------------|---------|
| 2,2'-methylene-bis(6-tert.-butyl-4-methylphenol) | 100 g   |
| Phthalazinone                                    | 5 g     |
| Polyvinyl butyral                                | 10 g    |
| Methanol                                         | 1000 ml |

60

The coated paper thus obtained was divided into two pieces. One of the pieces was subjected to heat pre-treatment at 100°C for 5 seconds by contacting a back surface thereof with a heating roller. Then, a negative image was printed thereon by using a blue luminescent lamp. After heating at 120°C for 5 seconds, a pure black positive image completely free from fog was obtained, the back being white. The other piece was ex-

65

posed to the light of 40 W day-light luminescent lamp (Toshiba FL-40 S.D.) to be used for interior illumination at a distance of 2 m for 2 hours prior to the heat pretreatment. Thereafter, heat pre-treatment, exposure and heat development were carried out in the same manner as above. In spite of the above 2 hours' exposure, a pure black image completely free from fog could be obtained.

#### EXAMPLE 6

100 Parts of the first coating dispersion used in Example 1 were prepared. The following components were added and dissolved thereto successively, immediately before the application.

|                                                  |        |
|--------------------------------------------------|--------|
| 2,2'-methylene-bis(6-tert.-butyl-4-methylphenol) | 1.7 g  |
| Phthalazinone                                    | 0.65 g |

The thus resulting coating solution was applied to a photographic base paper and dried. After heat pre-treatment, exposure and heat development in the same manner as in the preceding example, a black positive image could be obtained.

#### EXAMPLE 7

The second coating solution in Example 5 was replaced with the following coating composition containing the following spectral sensitizing dye:

|                                                  |         |
|--------------------------------------------------|---------|
| Second coating solution:                         |         |
| 2,2'-Methylene-bis(6-tert.-butyl-4-methylphenol) | 100 g   |
| Phthalazinone                                    | 5 g     |
| Acridine Yellow G (CI-46025)                     | 0.01 g  |
| Polyvinyl butyral                                | 10 g    |
| Methanol                                         | 1000 ml |

The coated paper thus obtained was subjected to heat pre-treatment at 100°C for 5 seconds by contacting the back surface thereof with a heating roller. After exposure to a light of 150 W tungsten lamp for enlargement at a distance of 30 cm for 5 seconds followed by heat development at 110°C for 5 seconds, a pure black positive image similar to that of Example 5 was obtained, the back being white.

#### EXAMPLE 8

On the surface of the coated paper prepared in the same manner as in Example 5, the following third coating solution containing a spectral sensitizing dye was applied.

|                                                                                        |         |
|----------------------------------------------------------------------------------------|---------|
| Third coating composition:                                                             |         |
| 1-carboxymethyl-5-[(3-ethyl-2(1)-benzoxazolidene)-ethylidene]-3-phenyl-2-thiohydantoin | 0.01 g  |
| Methanol                                                                               | 1000 ml |

After pre-treatment followed by exposure and then heat development in the same manner as in Example 7, a black positive image could be obtained.

The embodiments of the invention in which an exclusive property or privilege is claimed are defined as follows:

1. A heat-developable light-sensitive material comprising a silver salt of long chain fatty acid, an organic reducing agent and an organic carboxylic acid, to which a heat-pretreatment was effected so as to impart to the material an image-forming ability by activation.
2. A heat-developable light-sensitive material according to claim 1, in which said heat-pretreatment was effected at a temperature of 50° to 200°C.
3. A heat-developable light-sensitive material according to claim 1, in which said heat-pretreatment was effected at a temperature of 70° to 120°C and the change in optical density of the surface of the material during the heat-pretreatment is below 0.1.
4. A heat-developable light-sensitive material according to claim 1, in which 10 - 0.01 part by weight of the organic reducing agent and 10 - 0.01 part by weight of the organic carboxylic acid are used based on 1 part by weight of the silver salt of long chain fatty acid.
5. A heat-developable light-sensitive material according to claim 1, in which 1 - 1/10 mole of the organic reducing agent and 10 - 1/10 mole of the organic carboxylic acid are used based on 1 mole of the silver salt of long chain fatty acid.
6. A heat-developable light-sensitive material according to claim 1, in which a spectral sensitizing dye selected from the class consisting of cyanines, merocyanines, oxonols and acridines is incorporated in the material.
7. A heat-developable light-sensitive material according to claim 1, in which the silver salt is a silver salt of long chain fatty acid having 18 to 24 carbon atoms.
8. A heat-developable light-sensitive material according to claim 7, in which said silver salt is selected from silver behenate and silver stearate.
9. A heat-developable light-sensitive material according to claim 1, in which said carboxylic acid is a long chain fatty acid having 18 to 24 carbon atoms.
10. A heat-developable light-sensitive material according to claim 1, in which a binder is incorporated in the material.
11. A heat-developable light-sensitive material according to claim 10, in which a layer or layers containing the silver salt, the organic reducing agent, the carboxylic acid and the binder are provided on a support.
12. A process for the preparation of heat-developable light-sensitive materials which comprises the steps of providing a first coating layer comprising a dispersion of a silver salt of long chain fatty acid and an organic carboxylic acid on a support, then treating the surface of the layer with a solution containing an organic reducing agent, drying the same and subjecting it to a heat pretreatment at a temperature of 50° - 200°C in order to dissociate a part of the silver salt.
13. A process for forming an image which comprises the steps of applying a radiation energy to the material according to claim 1 in a pattern of the image for exposure and then heat-developing the same.
14. A reproducing material comprising a silver salt of long chain fatty acid, an organic reducing agent and an organic carboxylic acid which is light inactive before it is subjected to heat-pretreatment.
15. A process for imparting light-sensitivity, in which the material according to claim 14 is subjected to heat-

pretreatment to convert the material to a light-sensitive one.

16. A process for forming an image which comprises the steps of applying a thermal energy to the material

according to claim 14 in a pattern of the image, exposing the whole surface to radiation energy and then heat-developing the same.

\* \* \* \* \*

5

10

15

20

25

30

35

40

45

50

55

60

65